

Oct. 8, 1968

C. F. RALEY, JR.

3,405,039

MAGNESIUM STRUCTURES FOR STORING AND PURIFYING ARALKYL HALIDES

Filed Aug. 9, 1965



INVENTOR.  
Charles F. Raley, Jr.  
BY  
George R. Baker  
ATTORNEY

## 1

3,405,039

## MAGNESIUM STRUCTURES FOR STORING AND PURIFYING ARALKYL HALIDES

Charles F. Raley, Jr., Midland, Mich., assignor to The Dow Chemical Company, Midland, Mich., a corporation of Delaware

Filed Aug. 9, 1965, Ser. No. 478,455  
3 Claims. (Cl. 203—86)

## ABSTRACT OF THE DISCLOSURE

Method for handling and purification of chlorinated hydrocarbons such as methyl chloride, carbon tetrachloride, methyl chloroform, benzyl chloride, ethylbenzyl chloride, chloroethylbenzyl chloride or vinylbenzyl chloride consisting of conducting such acts in magnesium alloys which contain alloying ingredients of 0—9% by weight of aluminum, and up to 6% of at least one of manganese, thorium, zinc and zirconium.

The present invention relates to novel methods for handling chlorinated hydrocarbons. More particularly the present invention concerns the storage of chlorinated hydrocarbons such as methyl chloride, carbon tetrachloride, methyl chloroform, benzyl chloride, ethylbenzyl chloride, chloroethylbenzyl chloride or vinylbenzyl chloride in magnesium containers. In addition the present invention also concerns the purification of such chlorinated hydrocarbons in magnesium stills.

It is well known that Friedel-Crafts catalysts such as HCl or AlCl<sub>3</sub> cause rapid and sometimes explosive decomposition of many chlorinated hydrocarbons such as those set forth above. To forestall these undesirable decompositions these chlorinated hydrocarbons are usually prepared and stored in nickel equipment and containers, and are stabilized by the addition of chemical stabilizers. Further, the purification is carried out in glass-line equipment or nickel equipment to prevent degradation of the chemical.

It has now been found that certain magnesium alloys will not react with these halogenated hydrocarbons. One can employ an alloy containing aluminum in the amount of 0 to 9 percent by weight and minor amounts less than 6% by weight of manganese, thorium, zinc, or zirconium, these alloys have ASTM or SAE numbers as follows:

| SAE | ASTM      | Alloy         | Composition                  |
|-----|-----------|---------------|------------------------------|
| 52  | B 107-56T | AZ31B (AZ31C) | 3% Al; 1% Zn; Bal. Mg.       |
| 520 | B 107-56T | AZ61A         | 6.5% Al; 1% Zn; Bal. Mg.     |
| 523 | B 107-56T | AZ80A         | 8.5% Al; 0.5% Zn; Bal. Mg.   |
| 522 | B 107-56T | MIA           | 1.20% Mn; 0.14% Ca; Bal. Mg. |

The following examples illustrate the present invention but are not to be construed as limited except by the claims appended hereto:

## Apparatus and test methods for collection of storage data of aralkyl halides in magnesium alloy containers

Test cans were prepared from 0.072" Dowmetal AZ-31B, each to have a capacity about 800 cc. The top and bottom were welded in; the side seam was also welded. Some of the cans were equipped with tapered Dowmetal stoppers. In addition to the magnesium cans, cans were also fashioned in essentially the same manner employing nickel metal.

Both anhydrous and water-saturated test fluids were used. The wet fluids were prepared by thoroughly shaking the fluid with excess water and allowing the mixture to

## 2

stand until well separated before use. The wet fluids had a milky appearance.

The test results were obtained by examining the fluids visually and by measuring refractive index of the fluids before and after the test and obtain the increase or decrease by difference and, also, by visual examination of the containers after sawing them in half lengthwise. In this way, deterioration of the liquids and/or the containers could be observed.

The containers were stored in a walk-in hood in which steam was continually venting; the atmosphere was consequently quite humid. This would affect the open-container tests.

A summary of performance is given in Table I. It will be observed that in the three-month test in closed Mg cans, all the fluids except vinylbenzyl chloride (VBC) appeared to be little affected, although some color change occurred. The wet VBC has polymerized to a very viscous syrup, while the dry fluid still was about as fluid as SAE 20 oil (the viscosity of the VBC on starting was 1.89 cp. at 25° or about the same as Kerosine).

The condition of the interior of the containers was also observed. The cans containing the dry liquids were in excellent condition, while those containing wet liquids had all suffered attack to a greater or lesser degree, the can containing wet chloroethylbenzyl chloride (CEBC) being in the worst condition.

After six months exposure in Mg cans much the same picture was presented. The liquids, except for VBC were in good condition. The dry VBC had polymerized to a heavy syrup while the wet VBC had become a clear yellow polymer, slowly soluble in toluene.

The Mg containers, after six months, were about like the three-month ones except for a slight haziness after contact with the dry liquids.

Since the above tests are representative of the most severe storage conditions, another three-month test was run using anhydrous fluids and open containers, a condition which would be representative of a drum in use with the cap left off. Also, as a standard of comparison, the same test was run simultaneously using nickel containers.

Judging by the refractive indexes in this series of tests, none of the liquids had undergone significant decomposition. The VBC in magnesium containers had an excellent appearance, as did the ethylbenzyl chloride (EBC) in nickel and VBC in nickel. The EBC in magnesium was turbid but colorless while the CEBC in magnesium was turbid, light brown and had sediment present. In the case of CEBC in nickel, the liquid was clear but dark green, possibly indicating nickel in solution.

The appearance of the interior of the containers was noted. The magnesium cans all had light specks of corrosion in the vapor space, and a greater or lesser degree of corrosion around the upper rim. Except for the can containing EBC, which had a fairly heavy apple-green deposit in the liquid space, the nickel cans gave excellent results.

Finally, a severe-condition test was run on closed nickel containers, using water-saturated liquids. In all cases, the liquids after three months contained a separate aqueous phase. The indexes suffered little change, although the liquids showed turbidity and in two cases, color changes.

The nickel cans containing EBC and VBC performed well, with only slight discoloration, while the can containing CEBC had heavy red-brown deposits in the liquid space and yellow-brown deposits in the vapor space.

It was thus demonstrated that magnesium-alloy containers give excellent results when water was excluded from the system.

TABLE I

## LIQUIDS AFTER STORAGE

| Test conditions         | Liquid                | Additives, 100 p.p.m. | Increase (+) or decrease (-) in $n_D^{25}$ | Color <sup>4</sup> | Remarks <sup>5</sup> |
|-------------------------|-----------------------|-----------------------|--------------------------------------------|--------------------|----------------------|
| Mg cans sealed 3 months | EBC <sup>1</sup> dry  | t-butyl catechol      | 0.0000                                     | W.W.               |                      |
|                         | EBC wet               | (TBC)m-nitro-p-       | -0.0003                                    | W.W.               |                      |
|                         | CEBC <sup>2</sup> dry | cresol (MNPC)         | -0.0003                                    | Dk. Gr.            | S                    |
|                         | CEBC wet              | diphenyl amine        | -0.0002                                    | G.r. Yel.          | S                    |
|                         | VBC <sup>3</sup> dry  | (DPA).                | +0.0069                                    | Lt. Yel.           | T                    |
| Mg cans sealed 6 months | VBC wet               |                       | V.viscous                                  | W.W.               | S                    |
|                         | EBC dry               |                       | +0.0002                                    | Lt. Yel.           | S                    |
|                         | EBC wet               |                       | +0.0002                                    | W.W.               | S                    |
|                         | CEBC dry              |                       | +0.0003                                    | Gr.                | S                    |
|                         | CEBC wet              |                       | -0.0001                                    | Gr.                | S                    |
| Mg cans open 3 months   | VBC dry               |                       | V.viscous                                  | Yel.               |                      |
|                         | VBC wet               |                       | Solid                                      | Yel.               |                      |
|                         | EBC dry               |                       | +0.0006                                    | W.W.               | S                    |
|                         | CEBC dry              |                       | 0.0000                                     | Lt.Br.             | S                    |
|                         | VBC dry               |                       | +0.0002                                    | Yel.               |                      |
| Ni cans open 3 months   | EBC dry               |                       | +0.0005                                    | Lt. Yel.           |                      |
|                         | CEBC dry              |                       | 0.0000                                     | Dk. Gr.            |                      |
|                         | VBC dry               |                       | +0.0002                                    | Yel.               |                      |
| Ni cans sealed 3 months | EBC wet               |                       | +0.0001                                    | W.W.               | Dk. Gr. Aq. phase.   |
|                         | CEBC wet              |                       | -0.0002                                    | Dk. Gr.            | Do.                  |
|                         | VBC wet               |                       | 0.0001                                     | Yel.               | Do.                  |

<sup>1</sup> EBC—ethylbenzyl chloride, water white;<sup>2</sup> CEBC—chloroethylbenzyl chloride, yellow;<sup>3</sup> VBC—vinylbenzyl chloride, yellow;<sup>4</sup> W.W., water white; Dk., dark; Lt., light; Gr., green; Yel., yellow; Br., brown;<sup>5</sup> T—turbid; S—slight sediment observed.

## Example 2

The following example illustrates the utility of magnesium alloys for use in distillation equipment when purifying aralkyl halides.

The alloy of Dowmetal used was AZ31 since this is the most common alloy and is available in a wide variety of shapes, it would be expected to be the more widely employed of the alloys. A column 5 ft. high of 4" O.D. Dowmetal, equipped with a glass head and boiling flask was arranged for continuous distillation. The column was started up on chlorinator product, which is approximately a 50:50 mixture of ethylbenzyl chloride and chloroethylbenzyl chloride. The ethylbenzyl chloride was taken off overhead. After 143 hours of operation, the still was shut down and restarted as a flash still, taking chloroethylbenzyl chloride overhead. This operation was continued for an additional 811 hours and finally shut down when the feed was exhausted. During this run, samples were taken of the distillate and residue for magnesium analysis. From the results as shown in Table III it appears that there is an initial slight attack but that the metal becomes deactivated. The interior of the column was very clean after this run.

TABLE III.—MAGNESIUM CONTENT OF DISTILLATE AND RESIDUE FROM PART-DOWMETAL COLUMN

| Sample Description        | Hours of Operation | Percent Mg |
|---------------------------|--------------------|------------|
| Et benzyl Cl (overhead)   | 0                  | 0.0023     |
| ClEt benzyl Cl (residue)  | 0                  | 0.0027     |
| Et benzyl Cl (overhead)   | 60                 | 0.0119     |
| ClEt benzyl Cl (residue)  | 60                 | 0.0067     |
| Et benzyl Cl (overhead)   | 143                | 0.0022     |
| ClEt benzyl Cl (residue)  | 134                | 0.0034     |
| ClEt benzyl Cl (overhead) | 143                | 0.0022     |
| Do                        | 168                | 0.0042     |
| Residue                   | 168                | 0.0041     |
| ClEt benzyl Cl (overhead) | 567                | <0.0001    |
| Residue                   | 567                | <0.0001    |
| ClEt benzyl Cl (overhead) | 954                | <0.0001    |
| Residue                   | 954                | <0.0010    |

A second column was fabricated almost entirely from Dowmetal AZ31. The reboiler was a thermosyphon type, using a single tube heater. Due to the impossibility of using steam as a heating medium, a 4500 watt Dowtherm boiler was used to heat tri-isopropylbenzene, which was then circulated through the magnesium reboiler at 200° C. Flange fittings with poly tetrafluoro ethylene envelope asbestos gaskets were used to couple the iron boiler to the Dowmetal unit. The reboiler was equipped with a ball-joint residue take-off tube which fitted a glass socket in the receiver system. A flanged-in thermowell was centered in the heating zone. The unit was insulated with 1" pipe covering. The overall height of the reboiler was approximately 60".

The column section consisted of the original 5 ft. column, surmounted by a 3½ ft. extension, into which was welded a feed tube. This column was also packed with ½" Berl saddles.

The still head was composed of a 26" disengaging section, fitted with a thermowell and metal ball connection to fit a reflux tube, topped by a length of 2" OD x ¼" wall magnesium alloy AZ31B tubing bent into a 180° turn, with no welds breaking the continuity. The take-off end was surrounded by a water jacket, giving a condensing area of approximately 113 sq. in. A brace rod between the water jacket and the disengaging section prevented the bend from springing open when heated.

Water saturated with zinc chromate was used as the coolant. To avoid replenishing the chromate, the coolant was recycled, being in turn cooled by a stainless steel shell and tube heat exchanger using tap water.

To the take-off flange was attached a glass stream-splitter, with a magnetically operated swinging spout. With the magnet deactivated, the distillate was returned to the column by way of a U-trap and a reflux tube. The other take-off led to a glass receiver system.

The still was operated by charging a feed of vinylbenzyl chloride and chloroethylbenzyl chloride into the still column, heated to 200° C. Periodic samples were taken of the overhead and residue and analyzed for magnesium content. The results of the analysis are set forth below.

TABLE V.—MAGNESIUM CONTENT OF DISTILLATE AND RESIDUE FROM COMPLETE DOWMETAL COLUMN

| 55 | Sample description         | Hours of operation | Percent Mg |
|----|----------------------------|--------------------|------------|
|    | Vinyl benzyl Cl (overhead) | 33                 | <0.0001    |
|    | ClEt benzyl Cl (residue)   | 33                 | 0.0007     |
|    | Vinyl benzyl Cl (overhead) | 101                | 0.0001     |
|    | ClEt benzyl Cl (residue)   | 101                | <0.0001    |
| 60 | Vinyl benzyl Cl (overhead) | 151                | <0.0001    |
|    | ClEt benzyl Cl (residue)   | 151                | <0.0001    |
|    | Vinyl benzyl Cl (overhead) | 179                | <0.0001    |

It is thus obvious a magnesium alloy still can be employed to separate and purify chloroaromatics as effectively as the special materials of construction previously employed.

I claim:

1. A method for storing and shipping chlorinated aliphatic and chlorinated aralkyl hydrocarbons which normally undergo decomposition in the presence of aluminum when unstabilized selected from the group consisting of methyl chloride, carbon tetrachloride, methyl chloroform, benzyl chloride, ethylbenzyl chloride, chloroethylbenzyl chloride and vinylbenzyl chloride, which consists of containing the said liquid hydrocarbons in an un-

stabilized condition in containers of magnesium alloy having from 0 to 9% by weight Al, and minor amounts less than 6% by weight of at least one of the metals thorium, zinc, manganese and zirconium.

2. The method for distilling aralkyl and aliphatic chlorinated hydrocarbons which undergo decomposition or polymerization in the presence of aluminum selected from the group consisting of methyl chloride, carbon tetrachloride, methyl chloroform, benzyl chloride, ethylbenzyl chloride, chloroethylbenzyl chloride and vinylbenzyl chloride, which consists of conducting the distillation in stills of magnesium alloy having from 0 to 9% by weight Al, and minor amounts less than 6% by weight of at least one of the metals thorium, zinc, manganese or zirconium.

3. A still for purifying chlorinated hydrocarbons comprising a liquid-vapor zone having a vapor outlet at its top connected by a tubing to a condensing zone which is below the outlet of a reboiler associated with said liquid-vapor zone to deliver vapor and liquid in a heated condition to said vapor-liquid zone, all of said components consisting of magnesium alloy having from 0 to 9% by

5

10

15

20

weight Al, and minor amounts less than 6% by weight of at least one of the metals thorium, zinc, manganese and zirconium.

#### References Cited

#### UNITED STATES PATENTS

|           |         |                   |           |
|-----------|---------|-------------------|-----------|
| 1,932,474 | 10/1933 | Penhaligon        | 75-168    |
| 2,068,868 | 1/1937  | Pier et al.       | 196-133   |
| 2,314,024 | 3/1943  | Topping           | 75-168    |
| 2,870,094 | 1/1959  | Cathcart          | 260-652.5 |
| 2,849,430 | 8/1958  | Amos et al.       | 159-48    |
| 2,999,886 | 9/1961  | Crabb et al.      | 260-652.5 |
| 3,274,077 | 9/1966  | Hoffenberg et al. | 203-86    |
| 2,079,786 | 5/1937  | Beck              | 206-84    |

#### OTHER REFERENCES

C. S. Roberts: Magnesium and Its Alloys, pub. 1960, N.Y., pp. 159, 160, 202 and 203, relied upon.

WILBUR L. BASCOMB, Jr., *Primary Examiner.*